

R. J. McNITT.  
METHOD OF REDUCING METALS.  
APPLICATION FILED MAY 12, 1915.

1,214,808.

Patented Feb. 6, 1917.



Robert J. Mc. Nitt Inventor

By his Attorneys  
Mastick & Tucke

# UNITED STATES PATENT OFFICE.

ROBERT J. McNITT, OF NIAGARA FALLS, NEW YORK, ASSIGNOR TO THE ROESSLER & HASSLACHER CHEMICAL CO., OF NEW YORK, N. Y., A CORPORATION OF NEW YORK.

## METHOD OF REDUCING METALS.

1,214,808.

Specification of Letters Patent.

Patented Feb. 6, 1917.

Original application filed January 2, 1913, Serial No. 739,710. Divided and this application filed May 12, 1915. Serial No. 27,474.

*To all whom it may concern:*

Be it known that I, ROBERT J. McNITT, a citizen of the United States of America, residing at Niagara Falls, county of Niagara, and State of New York, have invented a certain new and useful Method of Reducing Metals, of which the following is a specification:

My invention relates to a new and useful 10 method of reducing metals from compounds containing the same and it refers particularly to the reduction of metals from their compounds by electrolyzing the same under pressure.

15 In my copending patent application Serial No. 739,710, filed January 2, 1913, of which this is a division, I broadly disclosed my invention of an improved method for the electrolytic reduction of metals consisting in carrying on the electrolysis under pressure, the pressure specifically described and claimed in the original application being that due to a gas compressed against the upper surface of the electrolyte. In 20 my said original application I stated that the same improvement in the electrolysis of metals could be secured by carrying on the electrolysis under the pressure due to a superimposed column of electrolyte which 25 method I shall now more fully explain by describing, as an example, the electrolysis of metallic sodium from molten sodium chlorid. I shall explain this form of my invention by reference to the accompanying 30 drawing, which is a vertical longitudinal section showing in rather a diagrammatic way one form of apparatus suitable for the purpose.

A indicates the anode which may be of 40 graphite or other suitable material. It is electrically connected with conductors B extending through the walls of the vessel. The cathode C, of any suitable material is shown as connected on its lower side with 45 a conductor D extending through the bottom of the vessel. The walls of the vessel may be formed of steel plates E lined on the inside with a layer of asbestos F, the space between said walls and the rear sides 50 of the anodes and above the said anodes being filled in with a suitable material such as brick work G, preferably fire-clay brick. The working chamber of the vessel extends from the bottom X up to the cover H.

Z indicates a bell of any suitable material, shown as somewhat larger in its lateral extension than the cathode C. 55

K represents a diaphragm of perforated metal extending from the lower rim on the bell Z downward between the anode and 60 cathode, the lower rim being shown as terminating a short distance from the upper edge of the cathode C.

Z' indicates a tube connected to the upper 65 part of the bell Z and passing through the cover H. A pipe N branches from the tube Z' and connects it to a receiver O which is provided with a valve O'. The pipe P serves to conduct away the gases generated 70 during the process and another pipe Q provided with a cover serves for charging the metallic compound (in the presumed instance, sodium chlorid) into the vessel.

In carrying out my invention I prefer to charge the apparatus with molten electrolyte to the requisite height. The height giving the most favorable results depends upon various conditions such as the nature and degree of purity of the electrolyte, the proximity of the fusing point of the electrolyte to the boiling point of the metal separated, the current density employed, and the shape and surface conditions of the electrodes. In the example cited the column of molten sodium chlorid should be 85 carried to such a height above the zone of electrolysis that it shall exert a pressure of at least one pound per square inch in 90 said zone of electrolysis. Electric current is then passed through the electrolyte, decomposing the same with liberation of chlorin gas at the anode, and metallic sodium at the cathode. The chlorin passes up 95 through the electrolyte, and escapes by way of the pipe P. The metallic sodium liberated at the cathode, rises into and is collected under the bell Z.

As the continuous electrolysis constantly increases the volume of metallic sodium within the bell, owing to the difference in 100 the specific gravity of the respective liquids the sodium rises in the bell and finally overflows through the pipe N into the receiver O.

Many modifications in the way of conducting the process described may be made, without departing from the nature of my 105 invention. For instance the form and con-

struction of the bell Z may be modified so as to allow the introduction of the cathode C and its conductor D from the top instead of through the bottom of the vessel. Other changes which may be desirable in the relative position of the electrodes may also be made. The metallic compound may be introduced in a solid instead of in a molten state; the high column of fluid exerting the pressure on the zone of electrolysis consists preferably of the molten electrolyte, but it may partly or even entirely be substituted by other suitable liquid substances. The vessel may be square or round or of any other suitable shape.

The apparatus hereinbefore described is well suited for the purposes of my invention for the production, for instance of metallic sodium from its compounds, preferably sodium chlorid, but other metals may be similarly obtained from their compounds and my invention is not limited to the use of the particular apparatus which I have described and illustrated.

25 I claim:

1. A method of reducing metallic compounds to their metals, consisting in subjecting the molten metallic compounds in the zone of electrolysis to comparatively great hydrostatic pressure during the electrolytic process.
2. A method of reducing metallic compounds to their metals by electrolysis, consisting in subjecting the molten metallic compounds in the zone of electrolysis to the pressure of a column of fluid high relative to the cross section of the electrolytic chamber and electrolyzing the metallic compounds under the pressure thus exerted.
3. A method of reducing metallic compounds to their metals by electrolysis, consisting in subjecting the molten metallic compounds in the zone of electrolysis to the pressure of a column of the molten metallic compound high relative to the cross section of the electrolytic chamber and then electrolyzing the same under the pressure thus exerted.
4. A method of reducing metallic com-

pounds to their metals by electrolysis, consisting in introducing said metallic compounds forming the electrolyte, in a molten state, into the electrolytic zone, superimposing a high column of said molten metallic compounds on the zone of electrolysis, passing the electric current through the bath of metallic compounds, separating the products generated at the electrodes as desired and controlling the applied pressure by the height of the column of the molten metallic compounds.

5. A method of reducing metallic sodium from its compounds, consisting in subjecting the molten sodium compound in the zone of electrolysis to the pressure of a column of fluid high relative to the cross section of the electrolytic chamber and then electrolyzing the sodium compounds under the pressure thus exerted.

6. A method of reducing metallic sodium from its compounds, consisting in subjecting the molten sodium compound, forming the electrolyte, in the zone of electrolysis to the pressure of a column of said molten sodium compound high relative to the cross section of the electrolytic chamber and electrolyzing the same under the pressure thus exerted.

7. A method of reducing metallic sodium from its compounds by electrolysis, consisting in introducing said sodium compound forming the electrolyte, in a molten state, into the electrolytic zone, superimposing a high column of the molten sodium compound on the zone of electrolysis, passing the electric current through the bath of said sodium compound, separating the products generated at the electrodes as desired and controlling the applied pressure by the height of the column of the molten sodium compound.

In testimony whereof I have signed this specification in the presence of two subscribing witnesses.

ROBERT J. McNITT.

Witnesses:

FRANK A. DUDLEY,  
H. W. CLARK.